

1

2,792,301

PROCESS OF MANUFACTURING FLINT OR LIKE PYROPHORIC MATERIAL IN EXTRUSION PRESSES

Walter Bungardt, Essen, Germany, assignor to Th. Goldschmidt A.-G. Chemische Fabriken, Essen, Germany, a German corporation

No Drawing. Application January 23, 1953,  
Serial No. 332,989

Claims priority, application Germany January 25, 1952

9 Claims. (Cl. 75—152)

This invention relates to the manufacture of flint or like pyrophoric material, in particular in rod formation as disclosed in my copending application Ser. No. 117,069, filed September 21, 1949, and now U. S. Patent No. 2,660,301.

Experiments have shown that if cerium-iron-alloys melted at a temperature between 1000° and 1200° C. are cast in molds of cast iron which are preheated to a temperature of approximately 600° to 700° C., the thus obtained cast ingots may be used as starting material for the manufacture of flints or like pyrophoric material in extrusion presses. As a source of cerium there may be employed misch metal which contains the metals of the rare earth group as main constituents and has a cerium content of about 45—55%.

Such material can then be subjected to the action of an extrusion press at temperatures ranging between 400° to 500° C. in order to obtain flint and like rods which are subsequently cut to conventional lengths, as required by the trade.

Depending upon the iron content of such alloys and depending upon the quality of the misch metal to be employed, shaping through extrusion presses necessitates quite different maximum press powers. If the iron content increases such press power must generally be considerably increased. In view of the different degrees of impurities which may be present in the misch metal compounds to be worked upon (said degrees depending upon the chemical composition of the ore employed), this press power may be considerably varied or influenced. The press power becomes higher the greater the degree of impurity which is present in the misch metal.

Extensive experiments have shown that it is possible to add or to admix to the misch metal-iron alloys such types of metals which have the same or a greater heat of formation when combined with oxygen (unit: gram-atom oxygen, than that of the cerium, so that the maximum press power required for the extrusion process may be considerably reduced.

This improving effect of the aforesaid metal additions is generally based on two conditions. In order to reduce the press power during extrusion formation under otherwise substantially equal outer pressure conditions, it appears necessary to reduce the inner friction of the particles within the ingot to be extruded. This can be achieved by eliminating from the ingot disturbing impurities, such as oxides or, possibly, nitrites, hydrides, carbides and similar impurities which are either contained in the misch metal itself or are admixed thereto by otherwise usual additions, such as for instance, iron. In the presence of certain definite metallic element additions and through substantially pure alloy effect a further reduction of the inner friction of the metal particles may be obtained, whereby the extrusion press power will be decreased.

In accordance with the present invention the pyrophoric misch metal-iron-alloys with an iron content of

2

4.5% to 40% are alloyed, in order to reduce the press power needed for carrying out the extrusion, with such metallic elements and in quantities of 0.3% to 10%, preferably 0.3% to 1%, said elements when compared with cerium having a substantially equal or larger heat of formation during transition into oxides. This effect has been found to be particularly noticeable in the case of titanium, the use of which brings about the desired decrease in the press power required to extrude the alloy even when the same has a quantity of tin, for example, incorporated therein. As is disclosed in the above-mentioned U. S. Patent No. 2,660,301, tin or another metal such as zinc, cadmium or magnesium, is usually employed as a hardness-increasing agent for the alloy and thus for the resulting flint so as to reduce wear and tear of the flint during use to a minimum. In addition, other metals may be employed, for the purpose of reducing the required press power, such as aluminum, magnesium, calcium, zirconium and beryllium, either singly or combined one with the other.

The following examples are given for the purpose of demonstrating the invention:

*Example I*

25 Misch metal obtained through bastnasite is alloyed with about 20.2% iron, 0.5% magnesium and 1% tin, the content of misch metal being approximately 78.4%. The hardness of this misch metal alloy in cast form amounts to 89 kg./mm.<sup>2</sup>. For the formation through extrusion 30 at a temperature of 480° C. a max. press power of 23.0 tons is required.

If to the amount of 78.4% of the same misch metal 19.5% iron, 0.5% magnesium, 1% tin, about 0.21% aluminum and about 0.60% titanium are added, then the 35 hardness of the cast alloy is increased to 97.8 kg./mm.<sup>2</sup>, the max. press power for the formation of the alloy in the extrusion press, however, is reduced by about 46%, now amounting to 12.5 tons.

*Example II*

40 If 78.4% misch metal obtained from monazite mineral sand is alloyed with 20% iron, 0.6% magnesium and 1% tin, the hardness of the cast alloy thus obtained amounts to 112 kg./mm.<sup>2</sup> and the required max. pressure for the 45 formation of the alloy in the extrusion press amounts to 33 tons. If 0.6% titanium is added to this alloy, then the hardness of such improved alloy is increased to 116 kg./mm.<sup>2</sup> while the max. press power for the formation of the alloy in the extrusion press is decreased by 42%, namely to 19 tons.

*Example III*

50 If 74.6% misch metal obtained from bastnasite is alloyed with 23.9% iron, 0.5% magnesium and 1% tin, the hardness of the resultant cast alloy amounts to 98.8 kg./mm.<sup>2</sup> and the max. press power amounts to 25 tons for working the alloy in the extrusion press.

If, however, 74.3% of the same misch metal is alloyed with 23.4% iron, 0.5% magnesium, 1% tin, 0.11% aluminum and 0.66% titanium, the hardness of the resultant 60 alloy is increased to 104 kg./mm.<sup>2</sup> and the max. press power is reduced by 40%, amounting to 15 tons for working the alloy in the extrusion press.

*Example IV*

65 If a misch metal obtained from bastnasite amounting to 70.6% is alloyed with 28% iron, 0.5% magnesium and 0.9% tin, the hardness of the cast alloy amounts to 108 kg./mm.<sup>2</sup> and the max. press power to 38 tons. If such misch metal amounting to 69.7% is alloyed with 70 28.1% iron, 0.5% magnesium, 1% tin, 0.12% aluminum and 0.7% titanium, the hardness of the alloy in cast state is increased to 120 kg./mm.<sup>2</sup>, the max. press

power being reduced for working of the alloy in the extrusion press by about 45%, namely, to 21 tons.

The addition of titanium, as well as of other metals as herein set forth with respect to the misch metal-iron-alloy with an iron content from 4.5% to 40% is of extreme practical importance for the manufacture of flint metal rods to be used for various purposes.

By reducing the max. press power in the extrusion press, practical working conditions for this alloy are greatly facilitated, while maintenance and durability of the dies and tools of the press are considerably simplified and improved.

Although specific embodiments of the invention have been described, it should be noted that the invention may be realized in modified form and adaptations of the arrangements herein disclosed may be made, as may readily occur to persons skilled in the art without constituting a departure from the spirit and scope of the invention as defined in the objects and in the appended claims.

Having thus described the invention, what is claimed as new and desired to be secured by Letters Patent is:

1. An alloy capable of being extruded at reduced press powers comprising about 60 to about 95.5 parts by weight of misch metal, about 4.5 to about 40 parts by weight of iron, and about .3 to about 1 part by weight of titanium having, upon conversion to the oxide, a heat of formation per gram atom of oxygen at least equal to that of cerium.

2. In the process of manufacturing pyrophoric flints by extrusion of ingots of an alloy containing a hardness-increasing agent, about 60 to 95.5 parts by weight of misch metal and about 4.5 to 40 parts by weight of iron, under pressure applied to said ingots at a temperature within the range of about 400° C. to about 500° C.; the step of incorporating in said alloy prior to extrusion of said ingots about 0.3 to about 1 part by weight of a metal having, upon conversion to the oxide thereof, a heat of formation per gram atom of oxygen at least equal to that of cerium, whereby the press power required to extrude said ingots is substantially reduced without adverse effect on the pyrophoric qualities of said flints made therefrom.

3. In the process of manufacturing pyrophoric flints by extrusion of ingots of an alloy containing a hardness-increasing agent, about 60 to 95.5 parts by weight of misch metal and about 4.5 to 40 parts by weight of iron, under pressure applied to said ingots at a temperature within the range of about 400° C. to about 500° C.; the step of incorporating in said alloy prior to extrusion

of said ingots about 0.3 to about 1 part by weight of titanium and another metal having, upon conversion to the oxide thereof, a heat of formation per gram atom of oxygen at least equal to that of cerium, whereby the press power required to extrude said ingots is substantially reduced without adverse effect on the pyrophoric qualities of said flints made therefrom.

4. The process according to claim 3, said other metal being aluminum.

10 5. The process according to claim 3, said other metal being calcium.

6. The process according to claim 3, said other metal being beryllium.

15 7. The process according to claim 3, said other metal being zirconium.

8. The process according to claim 3, said other metal being magnesium.

9. In the process of manufacturing pyrophoric flints by extrusion of ingots of an alloy containing a hardness-increasing agent, about 78.4 parts by weight of misch metal and about 20 parts by weight of iron, under pressure applied to said ingots at a temperature within the range of about 400° C. to about 500° C.; the step of incorporating in said alloy prior to extrusion of said

20 25 ingots about 0.3 to about 1 part by weight of titanium, whereby the press power required to extrude said ingots is substantially reduced by about 40 to 50% without adverse effect on the pyrophoric qualities of said flints made therefrom.

30

#### References Cited in the file of this patent

##### UNITED STATES PATENTS

|           |                  |               |
|-----------|------------------|---------------|
| 993,998   | Huber            | May 30, 1911  |
| 1,290,011 | Hirsch           | Dec. 31, 1918 |
| 2,023,498 | Winston          | Dec. 11, 1935 |
| 2,062,486 | Van Dusen et al. | Dec. 1, 1936  |
| 2,408,400 | Kent             | Oct. 1, 1946  |
| 2,660,301 | Bungardt         | Nov. 24, 1953 |

##### FOREIGN PATENTS

|         |               |                |
|---------|---------------|----------------|
| 49,215  | Switzerland   | Aug. 16, 1909  |
| 153,306 | Great Britain | Sept. 29, 1921 |
| 567,445 | Great Britain | Feb. 14, 1945  |
| 498,599 | Belgium       | Feb. 1, 1951   |

##### OTHER REFERENCES

Hackh's Chemical Dictionary, pub. by The Blakiston Co., Philadelphia, Pa., 3rd ed. 1944; page 541.